

## UNITED STATES PATENT OFFICE

MAXIMILIAN PAUL SCHMIDT AND RUDOLF ZAHN, OF WIESBADEN-BIEBRICH, GERMANY, ASSIGNORS TO KALLE & CO. AKTIENGESELLSCHAFT, OF BIEBRICH-ON-THE-RHINE, GERMANY

## LIGHT-SENSITIVE LAYERS AND PROCESS OF PREPARING THEM

No Drawing. Application filed October 23, 1929, Serial No. 401,964, and in Germany November 3, 1928.

The present invention relates to light sensitive layers and to a process of preparing them.

We have found that light sensitive layers can be produced with the aid of an arylazide which can be prepared in a known manner, for instance, by causing a diazo compound to react with sodium arylazide.

For the preparation of the light-sensitive layer the arylazide is dissolved in water or in an organic solvent, such as, for instance, alcohol; the solution is then applied on a base, for instance, paper or film. When the layers are exposed to light, dyestuffs are formed at those places where the light is allowed to react, whilst the places not exposed to light remain unaltered. Thus by exposure to light behind a negative a positive picture is obtained. The color of the picture depends on the particular arylazide chosen and it is possible to prepare pictures in all possible color tones, such as yellow, brown, red, violet to black by using arylazides with certain substituents.

The tones and the fastness of the pictures may be further modified by the addition of a base, an acid or a metallic salt used in diazo-type processes to the light-sensitive layer or to the washing baths. The arylazides may also be used in the presence of a colloidal body, for instance, gelatine, collodion and other bodies. Mixtures of azides may also be used. A stabilizer, such as for instance, glucose, tartaric acid and the salts thereof and aromatic sulpho acids, may also be added to the layer. After the exposure to light, a simple washing out with water or another suitable solvent is sufficient in order to render the pictures permanent.

The following examples serve to illustrate the invention, but they are not intended to limit it thereto, the parts being given by weight, except where otherwise specified.

1. A neutral or weakly alkaline aqueous solution of 3% strength obtained by causing diazo salicylic acid to react with sodium azide is spread upon paper. The paper is exposed to light under a negative and the picture thus obtained is washed with water. A brown positive copy is obtained. If the

light-sensitive solution is rendered weakly acid, a yellowish copy is obtained.

2. 2.5 parts of 4-azido-1,2-phenolcarboxylic acid are dissolved in 50 parts by volume of water with the addition of just the required quantity of caustic soda solution. 0.3 parts of boric acid and 0.6 parts of tartaric acid are added to the solution. The azido-salicylic acid which will have partly separated out is again dissolved with diluted caustic soda solution. The gelatine layer of the paper is impregnated with the solution obtained. After exposure to light under a negative and subsequent washing, pictures of a brown tone are obtained. Instead of impregnating the gelatine layer, the 4-azido-salicylic acid may also be applied upon the paper in the form of a gelatine emulsion.

3. 2 parts of 4-azido-1,2-phenolcarboxylic acid are dissolved in 25 parts by volume of water with the addition of some ammonia. The solution thus obtained is mixed with 0.5 parts of copper sulfate. Any portions which may separate out are again dissolved by adding some caustic soda solution. If this solution is applied on barium paper, allowed to dry and exposed to light under a negative, a positive picture is obtained, which after the washing operation has a brownish-yellow tone.

If a paper prepared according to Example 3, in which the copper sulfate is replaced by 0.5 parts of zinc chloride is employed, then by working according to the same method, pictures of a brownish-violet tone are obtained. If the same weight of titanic oxalate be substituted for copper sulfate, pictures of a brownish-red tone are obtained by working in a similar manner. If instead of the copper sulfate 0.7 parts of nickel chloride are used, dark black tones are obtained on gelatine paper.

4. 1 part of para-azidodiphenylamine carboxylic acid of the formula:



is dissolved with some diluted caustic soda solution in 25 parts by volume of water; 100

the solution thus obtained is applied on paper. After exposure to light under a negative and subsequent washing with water, pictures of a brownish-yellow tone are obtained.

5. 4 parts of 4-azido-1,2-phenolcarboxylic acid are dissolved in 50 parts by volume of water together with 1.3 parts of azidodiphenylamine carboxylic acid and 0.4 parts of glucose with the addition of some ammonia. Gelatine paper is rendered sensitive to light by means of this solution and the paper is then exposed to light under a negative. According to the length of time during which the pictures are exposed to light, positive pictures are obtained, the tones of which vary from dark brown to black.
6. 1 part of 1-azido-2-chloro-4-dimethylamino-benzene is dissolved in 25 parts by volume of water with the addition of some dilute hydrochloric acid. When the solution thus obtained is applied on paper, positive pictures of brownish-orange tones are obtained after exposure to light under a negative and subsequent washing.
25. 7.2 parts of 4-para-tolyl-sulfonyl-amino-1-azido-benzene of the formula:



30 are dissolved with some dilute caustic soda solution in 20 parts by volume of water. The papers impregnated with the solution thus obtained yield, after exposure to light under a negative and subsequent washing, positive pictures of brownish yellow tones.

The above named azido compound may also be employed without the addition of alkali by applying it in an alcoholic solution on paper. The pictures obtained by exposure to light under a negative must in this case be washed with alcohol in order to remove the non-used azido compound.

8. 2 parts of para-tolyl-sulfo-3-amino-1-azido-benzene are dissolved in 20 parts by 45 volume of water with the addition of some dilute caustic soda solution. The solution thus obtained is applied on paper. After exposure to light under a negative and washing with water, positive pictures of yellow 50 tones are obtained.

9. 1 gram of the sodium salt of the diazidodiphenylamine carboxylic acid of the formula:



is dissolved in 20 c. c. of alcohol of 20 per cent strength and applied on a paper which 60 has been covered with a gelatine layer. After drying and exposing said paper to light under a negative, a positive picture of a brown shade is obtained, which is washed with diluted alcohol in order to remove the 65 unaltered azido compound.

We claim:

1. Process of preparing light-sensitive layers upon a suitable base, which comprises applying an aryl-azide upon said base.

2. Process of preparing light-sensitive layers upon a suitable base, which comprises applying a substituted arylazide upon said base.

3. Process of preparing light-sensitive layers upon a suitable base, which comprises applying a compound of the following formula:



wherein the X's stand for hydrogen atoms some of which may be substituted by OH, COOH, N<sub>3</sub>, halogen, aryl, aralkyl, oxalkyl, alkyl, an amino group substituted or not or a sulfo group upon said base.

4. Process of preparing light-sensitive layers upon a suitable base, which comprises applying a compound of the following formula:



wherein one X stands for hydroxy or amino group substituted or not and the other X's stand for hydrogen atoms some of which may be substituted by OH, COOH, N<sub>3</sub>, halogen, aryl, alkyl, aralkyl, oxyalkyl or a sulfo group upon said base.

5. Process of preparing light-sensitive layers upon a suitable base, which comprises applying a compound of the following formula:



wherein one X may stand for COOH and one X for OH and the other X's for H upon said base.

6. Process of preparing light-sensitive layers upon a suitable base, which comprises applying a compound of the following formula:



upon any desired base.

7. Process of preparing light-sensitive layers upon a suitable base, which comprises applying an arylazide and a metallic salt used in the diazo-type process upon said base.

8. Process of preparing light-sensitive layers upon a suitable base, which comprises applying a compound of the following formula:



wherein one X stands for hydroxy or amino

group substituted or not and the other X's stand for hydrogen atoms some of which may be substituted by OH, COOH, N<sub>3</sub>, halogen, aryl, alkyl, aralkyl, oxyalkyl or a sulfo group and a metallic salt used in the diazo-type process upon said base.

9. Process of preparing light-sensitive layers upon a suitable base, which comprises applying an arylazide, a metallic salt used in the diazo-type process and a colloid upon said base.

10. Process of preparing light-sensitive layers upon a suitable base, which comprises applying an arylazide, a metallic salt used in the diazo-type process and gelatine upon said base.

11. As new products, light-sensitive layers containing an arylazide.

12. As new products, light-sensitive layers containing a substituted arylazide.

13. As new products, light-sensitive layers containing a compound of the following general formula:



30 wherein the X's stand for hydrogen atoms some of which may be substituted by OH, COOH, N<sub>3</sub>, halogen, aryl, alkyl, aralkyl, oxyalkyl, an amino group substituted or not or a sulfo group.

35 14. As new products, light-sensitive layers containing a compound of the following formula:



40 wherein one X stands for hydroxy or amino group substituted or not and the other X's stand for hydrogen atoms some of which may be substituted by OH, COOH, N<sub>3</sub>, halogen, aryl, alkyl, aralkyl, oxyalkyl or a sulfo group.

45 15. As new products, light-sensitive layers containing a compound of the following formula:



50 wherein one X may stand for COOH and one X for OH and the other X's for H.

55 16. As new products, light-sensitive layers containing a compound of the following formula:



60 17. As new products, light-sensitive lay-

ers containing an arylazide and a metallic salt used in the diazo-type process.

18. As new products, light-sensitive layers containing a compound of the following formula:



70 wherein one X stands for hydroxy or amino group substituted or not and the other X's stand for hydrogen atoms some of which may be substituted by OH, COOH, N<sub>3</sub>, halogen, aryl, alkyl, aralkyl, oxyalkyl or a sulfo group and a metallic salt used in the diazo-type process.

75 19. As new products, light-sensitive layers containing an arylazide, a metallic salt used in the diazo-type process and a colloid.

80 20. As new products, light-sensitive layers containing an arylazide, a metallic salt used in the diazo-type process and gelatine.

85 In testimony whereof, we affix our signatures.

90 MAXIMILIAN PAUL SCHMIDT.  
RUDOLF ZAHN.

75

80

85

90

95

100

105

110

115

120

125

130